



US005536633A

**United States Patent**

[19]

**Lok**[11] **Patent Number:** **5,536,633**[45] **Date of Patent:** **Jul. 16, 1996**

[54] **HEAT STABILIZED SILVER CHLORIDE PHOTOGRAPHIC EMULSIONS CONTAINING SULFUR DONORS AND SULFINATE COMPOUNDS**

[75] Inventor: **Roger Lok**, Rochester, N.Y.

[73] Assignee: **Eastman Kodak Company**, Rochester, N.Y.

[21] Appl. No.: **384,200**

[22] Filed: **Feb. 6, 1995**

**Related U.S. Application Data**

[63] Continuation of Ser. No. 160,016, Nov. 30, 1993, abandoned.

[51] **Int. Cl.<sup>6</sup>** ..... **G03C 1/015; G03C 1/34**

[52] **U.S. Cl.** ..... **430/569; 430/607; 430/611; 430/613; 430/614**

[58] **Field of Search** ..... **430/600, 603, 430/607, 611, 613, 614, 569**

**[56] References Cited****U.S. PATENT DOCUMENTS**

|           |         |                    |         |
|-----------|---------|--------------------|---------|
| H706      | 11/1989 | Takahashi et al.   | 430/551 |
| 2,057,764 | 10/1936 | Brunken            | 430/607 |
| 2,385,762 | 9/1945  | Mueller            | 430/607 |
| 2,394,198 | 2/1946  | Mueller            | 430/607 |
| 2,440,110 | 4/1948  | Mueller            | 430/607 |
| 2,440,206 | 4/1948  | Mueller            | 430/607 |
| 3,042,521 | 7/1962  | Dersch et al.      | 430/66  |
| 3,301,678 | 1/1967  | Humphlett et al.   | 430/61  |
| 3,466,173 | 9/1969  | Ishikawa et al.    | 430/596 |
| 3,615,534 | 10/1971 | Tajima et al.      | 430/67  |
| 3,759,901 | 9/1973  | Lincoln et al.     | 260/240 |
| 3,880,864 | 4/1975  | Lincoln et al.     | 260/286 |
| 4,245,033 | 1/1981  | Eida et al.        | 430/353 |
| 4,396,707 | 8/1983  | von Konig et al.   | 430/446 |
| 4,410,619 | 10/1983 | Kubbota et al.     | 430/234 |
| 4,451,557 | 5/1984  | Lok et al.         | 430/505 |
| 4,511,644 | 4/1985  | Okamura et al.     | 430/219 |
| 4,620,205 | 10/1986 | Iiyama et al.      | 346/204 |
| 4,770,987 | 9/1988  | Takahashi et al.   | 430/546 |
| 4,780,404 | 10/1988 | Sills et al.       | 430/572 |
| 4,859,580 | 8/1989  | Aono et al.        | 430/617 |
| 4,914,015 | 4/1990  | Philip, Jr. et al. | 430/572 |
| 4,939,072 | 7/1990  | Morigaki et al.    | 430/372 |
| 4,962,016 | 10/1990 | Chino et al.       | 430/603 |
| 5,006,448 | 4/1991  | Szajewski et al.   | 430/505 |
| 5,006,665 | 4/1991  | Rody et al.        | 549/28  |
| 5,043,259 | 8/1991  | Arai               | 430/596 |
| 5,070,007 | 12/1991 | Rody et al.        | 430/551 |
| 5,070,008 | 12/1991 | Maekawa et al.     | 430/567 |
| 5,082,766 | 1/1992  | Nishijima et al.   | 430/551 |
| 5,084,376 | 1/1992  | Suda et al.        | 430/617 |
| 5,091,294 | 2/1992  | Nishijima et al.   | 430/505 |
| 5,110,719 | 5/1992  | Shuto et al.       | 430/569 |

5,328,820 7/1994 Klaus et al. ..... 430/607

**FOREIGN PATENT DOCUMENTS**

|           |         |                         |           |
|-----------|---------|-------------------------|-----------|
| 0122125A1 | 10/1984 | European Pat. Off. .... | G03C 1/06 |
| 138622    | 4/1985  | European Pat. Off. .... |           |
| 447105    | 3/1988  | European Pat. Off. .... |           |
| 267483    | 5/1988  | European Pat. Off. .... |           |
| 294149    | 12/1988 | European Pat. Off. .... |           |
| 297804    | 1/1989  | European Pat. Off. .... |           |
| 305926    | 3/1989  | European Pat. Off. .... |           |
| 327272    | 9/1989  | European Pat. Off. .... |           |
| 349286    | 1/1990  | European Pat. Off. .... |           |
| 358170    | 3/1990  | European Pat. Off. .... |           |
| 447647    | 9/1991  | European Pat. Off. .... |           |
| 463639    | 1/1992  | European Pat. Off. .... |           |
| 3307506   | 9/1984  | Germany .               |           |
| 54-069428 | 6/1979  | Japan .                 |           |
| 55-144236 | 11/1980 | Japan .                 |           |
| 55-142331 | 11/1980 | Japan .                 |           |
| 60-178455 | 9/1985  | Japan .                 |           |
| 61-261737 | 11/1986 | Japan .                 |           |
| 62-270949 | 11/1987 | Japan .                 |           |
| 62-299963 | 12/1987 | Japan .                 |           |
| 63-37349  | 2/1988  | Japan .                 |           |
| 63-44650  | 2/1988  | Japan .                 |           |
| 63-37348  | 2/1988  | Japan .                 |           |
| 63-037348 | 2/1988  | Japan .                 |           |
| 63-037349 | 2/1988  | Japan .                 |           |
| 63-044650 | 2/1988  | Japan .                 |           |
| 1-196034  | 8/1989  | Japan .                 |           |
| 1-196050  | 8/1989  | Japan .                 |           |
| 2-020857  | 1/1990  | Japan .                 |           |
| 2-033141  | 2/1990  | Japan .                 |           |
| 2-148031  | 6/1990  | Japan .                 |           |
| 2-148033  | 6/1990  | Japan .                 |           |
| 2-161423  | 6/1990  | Japan .                 |           |
| 2-301744  | 12/1990 | Japan .                 |           |
| 3-033842  | 2/1991  | Japan .                 |           |
| 3-041438  | 2/1991  | Japan .                 |           |
| 1308938   | 3/1973  | United Kingdom .        |           |

*Primary Examiner*—Janet C. Baxter

*Attorney, Agent, or Firm*—Sarah Meeks Roberts

**[57] ABSTRACT**

A silver halide photographic element comprising a silver halide emulsion which is greater than 50 mole % silver chloride, said emulsion being in reactive association with a sulfur donating compound, and a sulfinate compound represented by Formula (I)

$Z-SO_2M^1$  (I)

wherein Z is a non-metallic aryl, alkyl or heterocyclic group, and M is a cationic counter ion;

and wherein the sulfur donor is not a thiosulfonate or a diamino disulfide; and a method of making the emulsion.

**16 Claims, No Drawings**

**HEAT STABILIZED SILVER CHLORIDE  
PHOTOGRAPHIC EMULSIONS  
CONTAINING SULFUR DONORS AND  
SULFINATE COMPOUNDS**

This is a Continuation of application Ser. No. 08/160,016, filed November 1993, now abandoned.

**FIELD OF THE INVENTION**

This invention relates to the use of addenda in silver halide photographic elements to improve heat stability.

**BACKGROUND OF THE INVENTION**

Photofinishers that use photosensitive paper to produce color prints desire short processing times in order to increase output. One way of obtaining rapid processing is to accelerate the development time by increasing the chloride content of the emulsions used in the photographic paper. However, as the chloride content of a photographic emulsion is increased, it becomes more difficult to obtain good invariant photosensitivity.

One of the problems with silver chloride emulsions is their severe propensity to storage deterioration. Photographic emulsions that have a high silver chloride content are prone to fog increase due to high temperature and humidity during storage. These changes may vary from layer to layer resulting in color imbalance and a loss of quality of the print material. Attempts have been made to reduce fog formation during storage by addition of inhibitory agents to the silver halide emulsions. For example, U.S. Pat. Nos. T866,036; 2,440,110; 3,043,696; 3,057,725; 3,226,232; 3,397,986; 3,447,925; and 3,761,277 describe the addition of organic disulfides to silver halide emulsions to lessen the tendency towards fog growth.

High chloride content color print paper also has an undesirable sensitivity to temperature changes during exposure. For example, when the temperature upon exposure rises due to heat from the exposing element during printing, the print density changes if the printing conditions are left at the initial set values. This may result in prints whose densities are different from those exposed at the normal temperature. This density difference contributes to print variability and is not acceptable to photofinishers. Very often, an increase in temperature during exposure of the paper may result in a selective increase in speed in one layer, for instance the cyan layer, over another light sensitive layer such as the magenta layer. This results in improper color balance of the color print, and requires the photofinisher to readjust his printing conditions in order to compensate for this density fluctuation. This results in a loss in operating efficiency.

This deficiency in the use of high silver chloride color paper material is recognized in the art. In particular, EP 0 367,227 (1988) discusses reducing heat sensitivity by employing certain spectral sensitizing dyes in combination with mercapto azoles. However, these dye structures have not proved to be entirely satisfactory in terms of minimizing thermal sensitivity while still maintaining optimal sensitization efficiency. EP 0 325,235 describes using iron ion donating compounds in high chloride photographic elements to reduce their change in sensitivity due to exposure at elevated temperature. Despite these attempts to address the thermal problem, no solution has been found which completely eliminates the above concerns.

U.S. Pat. No. 5,043,259 describes using alkyl and aryl disulfonates in the formation of pre-fogged direct positive silver halide emulsions. U.S. Pat. No. 4,939,072 describes using sulfonates as storage stability improving compounds in color photographs. U.S. Pat. No. 4,770,987 describes using sulfonates as anti-staining agents along with a magenta coupler in silver halide materials. EP 0 463,639, describes using sulfinic acid derivatives as dye stabilizers. U.S. Pat. No. 4,410,619 describes using a sulfinic acid salt to treat a paper base to prevent discoloration of the photographic material. U.S. Pat. No. 3,466,173 describes using aromatic sulfonates as stabilizers in a direct positive photographic material. EP 0 267,483 describes adding sulfonates during the sensitization of silver bromide emulsions. Similarly, GB 1,308,938 describes using sulfonates during processing of a silver halide photographic material to minimize discoloration of the image tone. U.S. Pat. No. 2,057,764 describes sulfonates as having fog reducing properties.

U.S. Pat. No. 5,110,719 describes using the combination of thiosulfonates with sulfonates and nucleating agents in a direct positive internal latent image core/shell chlorobromide emulsion. U.S. Pat. No. 3,615,534 describes using a combination of iodate ions and sulfonates to prevent yellow fog in silver halide materials. WO 92/12,462 describes using thiosulfonates and sulfonates in controlling speed increase on incubation of color photographic materials. JP 3,208,041 describes using the combination of thiosulfonates with sulfonates in the sensitization of chloride emulsions for color paper. U.S. Pat. No. 2,440,206 describes using the combination of sulfonates along with small amounts of polythionic acids to stabilize photographic emulsions against fog growth. U.S. Pat. No. 2,440,110 describes using the combination of sulfonates with aromatic or heterocyclic polysulfides in controlling fog growth. U.S. Pat. No. 2,394,198 describes using sulfonates with thiosulfonates in stabilizing silver halide emulsions. The use of sulfonates has been described as reducing stain in photographic paper when used in combination with sulfonates in U.S. Statutory Invention Registration H706, and in EP 0 305,926. U.S. Pat. No. 2,385,762 describes using a combination of diamino polysulfides and sulfonates or seleninates to stabilize silver halide emulsions. U.S. application Ser. No. 07/890,884 describes using diamino disulfides and sulfonates to reduce the thermal sensitivity of high chloride emulsions.

Compounds with labile sulfur moieties have been extensively used as sensitizers of silver halide emulsions. Their use and mechanism of action have been discussed in the photographic art such as by Pouradier, J. Properties of Gelatin in Relation to Its Use in the Preparation of Photographic Emulsions; James, T. H. Ed.; The Theory of the Photographic Process, 4th ed.; Macmillan: New York, 1977, Chapter 2; by Duffin, G. F. Photographic Emulsion Chemistry; Focal: London, 1966, Chapter 2 and by Mueller, F. W. H. in The Photographic Emulsion, Sturge, J. M. Ed.; Neblette's Handbook of Photographic and Reprography, 7th ed.; Van Nostrand Reinhold: New York, 1977, Chapter 2. Common among these labile sulfur compounds are thionates, thioureas, thiosulfates, isothiocyanates and sulfur containing amino acids such as cystine.

Elemental sulfur is known to be photographically active as described in EP 0 447,105; EP 0 297,804; EP 0 294,149 (AgCl); EP 0 327,272; EP 0 349,286; JP 2,161,423; JP 2,148,033; JP 2,148,031; JP 2,146,036; JP 2,033,141; JP 2,020,857; JP 2,301,744; JP 1,196,050; JP 1,196,034; DE 3,902,711; and U.S. Pat. No. 4,962,016.

Thiatriazoles have been used as supersensitizers for silver halide photographic materials as described in U.S. Pat. No.

4,914,015 (substituted thia and oxa thiatriazoles in red and infrared spectrally sensitized emulsions); U.S. Pat. No. 4,780,404 (amino thiatriazoles); EP 0 447,647 (arylaminothiatriazoles substituted with at least one electron-withdrawing group); and JP 3,033,842 and JP 3,041,438, (thiatriazoles as supersensitizers in red sensitized silver halide emulsions). JP 63/37,348 describes using thiatriazoles in silver chloride emulsions to obtain a low D-min photographic material. JP 63/44,650 and JP 63/37,349 describe a high storage stability material. U.S. Pat. No. 5,070,008 describes using thiatriazoles in silver chloride emulsions with iridium and acidic conditions for formation of AgCl grains. JP 80/142,331 describes using a thiatriazole in a photothermographic paper to reduce fog. U.S. Pat. No. 5,006,448 describes using a thiatriazole as an inhibitor fragment that is released for improving interimage effects.

Pyrazolopentathiepins have been described as fungicides or as sulfur sensitizers in photographic emulsions in EP 0 138,622. In JP 62/299,963 thiepin is mentioned as an example of a class of compounds used for the preparation of silver halide emulsions which comprises at least 50 mol% of silver bromide.

U.S. Pat. No. 4,620,205 discloses the use of dithiodialkylamines as decolorizing agents in a two-color thermosensitive recording material. In JP 54/69,428 and JP 55/144,236 dithiodialkylamines are alleged to sensitize silver bromide emulsions.

U.S. Pat. No. 4,960,689 describes using thiosulfonates in the finish in high Cl emulsions. Aromatic dithiosulfonic acids are described in U.S. Pat. No. 5,009,992 as supersensitizers in an IR-sensitive high Cl emulsion.

There remains a continuing need for an effective means for stabilizing high chloride emulsions against thermal changes.

## SUMMARY OF THE INVENTION

This invention provides a silver halide photographic element comprising a silver halide emulsion which is greater than 50 mole % silver chloride, said emulsion being in reactive association with a sulfur donating compound and a sulfinate compound represented by Formula (I)



wherein Z is a non-metallic aryl, alkyl or heterocyclic group, and M is a cationic counter ion; and wherein the sulfur donor is not a thiosulfonate salt or a diamino disulfide. This invention further provides a method of making the above described photographic emulsion.

The high chloride silver halide photographic elements of this invention exhibit very little variation in sensitivity upon changes in printing temperatures, while maintaining high resistance to storage changes. This allows for high quality prints without the need for constant readjustment of printing conditions during processing.

## DETAILED DESCRIPTION OF THE INVENTION

The sulfur donating compounds of this invention are those materials that extrude elemental sulfur on decomposition. Elemental sulfur is a form of sulfur that is zero valent and non-ionic. It is generally, but not always, expelled from the parent compound through a thermal process. That is, a myriad of other reactions, such as catalysis, and/or hydrolysis may take place, with the end result being that elemental

sulfur is extruded from the parent molecule, sometimes known as the sulfur precursor. These compounds have been extensively reviewed in the published literature, see Loudon, J. D. *The Extrusion of Sulfur*, Kharasch, N. K. Ed. Organic Sulfur Compounds, Pergamon: Oxford, 1961, Vol. 1, p. 299; Stark, B. P. and Duke, A. J. *Extrusion Reactions*, Pergamon: Oxford, 1967, p. 91; Radl, S. *Janssen Chim Acta*, 1987, 5, 3; Guziec, F. S. Jr and Sanfilippo, L. J. *Tetrahedron*, 1988, 44, 6241 and in Williams, C. R. and Harpp, D. N. *Sulfur Reports*, 1990, 10 (2), 103-191. Many of these compounds release elemental sulfur near or slightly above room temperature while others require temperatures as high as 200° C. or above. Still others require, in addition to high heat, presence of a trace metal for catalysis of the extrusion reaction. The preferred compounds of this invention are the ones that do not require a high temperature for extrusion, nor a specific catalyst or solvent, even though a catalytic reaction may take place in the silver halide emulsion to facilitate the extrusion reaction. More preferable are the compounds that will extrude sulfur below 200° C., and are stable at room temperature.

Examples of such sulfur donating compounds are certain disulfides, polysulfides, bis-alkylamino disulfides, sulfenic sulfonic thioanhydrides, thiosulfonate salts, aminothiosulfonates, acylmethylmercapto azoles or azonium salts, thiazepines, thiepins, 1,4-dithiins, 1,2-, 1,3-, or 1,4-thiazines, 1,4,2-dithiazines, 1,3,4-, 1,2,6-, 1,3,5-thiadiazines, dihydro derivatives of dithiazines or thiadiazines, and 1,2,3,4-thiatriazoles. Vulcanizing agents such as those discussed by Porter, M. in *Vulcanization of Rubber*; Oae, S. Ed.; Organic Chemistry of Sulfur; Plenum: New York, 1977, Chapter 3, and by Hofmann, W. *Vulcanization and Vulcanizing Agents*; Palmerton: New York, 1967 may also be effective. They include thiuram tetrasulfides, benzothiazolyl-2-N-dithiomorpholide, and di-morpholino disulfide. Elemental sulfur when appropriately dissolved in alcoholic solvents may also be useful. The following classes of sulfur donating compounds are particularly useful.

The acylmethylmercapto azonium salts are represented by Formula (A)



In the above structure,  $Z^1$  contains the atoms necessary to form either a five or six-membered fused or non-fused heterocyclic ring. Preferred heteroatoms are nitrogen, oxygen and sulfur. Examples of suitable heterocyclic groups are pyrrole, pyridine, picoline, piperidine, morpholine, pyrrolidine, oxazole, thiazole, imidazole, selenazole, tellurazole, triazole, tetrazole, thiadiazole, and oxadiazole.  $R^1$  and  $R^2$  are substituted or unsubstituted alkyl or aryl groups, more preferably, they are alkyl groups having 1 to 20 carbon atoms, with 1 to 6 carbon atoms being most preferred, or aryl groups having 6 to 10 carbon atoms, with 6 carbon atoms being most preferred. Examples of suitable substituents include alkyl groups (for example, methyl, ethyl, hexyl), fluoroalkyl groups (for example, trifluoromethyl), alkoxy groups (for example, methoxy, ethoxy, octyloxy), aryl groups (for example, phenyl, naphthyl, tolyl), hydroxy groups, halogen atoms, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl

groups (for example, methylsulfonyl, phenylsulfonyl), acylamino groups, sulfonylamino groups, acyloxy groups (for example, acetoxy, benzoxy), carboxy groups, cyano groups, sulfo groups, and amino groups. Preferred are simple alkyl groups.

$R^3$  is H, or an alkyl or aryl group as described for  $R^1$  and  $R^2$  and each may be further substituted as described for  $R^1$  and  $R^2$ . Q is an anion which may be, for example, a halide, a perchlorate, a hexafluorophosphate, a tetrafluoroborate, an organic carboxylate or a sulfonate. Examples of these of salts are shown below:



The thiepins are represented by Formula (B).



$R^4$ ,  $R^5$ ,  $R^6$ ,  $R^7$ ,  $R^8$ , and  $R^9$  are independently H or substituted or unsubstituted alkyl or aryl groups.  $R^4$ ,  $R^5$ ,  $R^6$ ,  $R^7$ ,  $R^8$ , and  $R^9$  together may form fused rings. Preferably, the alkyl groups contain 1 to 20 carbon atoms, with 1 to 6 carbon atoms being most preferred, and the aryl groups contain 6 to 10 carbon atoms, with 6 carbon atoms being most preferred. Examples of suitable substituents include alkyl groups (for example, methyl, ethyl, hexyl), fluoroalkyl groups (for example, trifluoromethyl), alkoxy groups (for example, methoxy, ethoxy, octyloxy), aryl groups (for example, phenyl, naphthyl, tolyl), hydroxy groups, halogen atoms, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl groups (for example, methylsulfonyl, phenylsulfonyl), acylamino groups, sulfonylamino groups, acyloxy groups (for example, acetoxy, benzoxy), carboxy groups, cyano groups, sulfo groups, and amino groups. Preferred are hydroxy groups.

Examples of specific thiepin compounds are shown below.



The 1,2,3,4-thiatriazoles are represented by Formula (C) below.



$R^{10}$  is a substituted or unsubstituted alkyl or aryl group, more preferably, an alkyl group having 1 to 20 carbon atoms, with 1 to 6 carbon atoms being most preferred, or an aryl group having 6 to 10 carbon atoms, with 6 carbon atoms being most preferred. Examples of suitable substituents include alkyl groups (for example, methyl, ethyl, hexyl), fluoroalkyl groups (for example, trifluoromethyl), alkoxy groups (for example, methoxy, ethoxy, octyloxy), aryl groups (for example, phenyl, naphthyl, tolyl), hydroxy groups, halogen atoms, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl groups (for example, methylsulfonyl, phenylsulfonyl), acylamino groups, sulfonylamino groups, acyloxy groups (for example, acetoxy, benzoxy), carboxy groups, cyano groups, sulfo groups, and amino groups. Preferred are hydroxy groups.

$n$  may be 0 or 1. When  $n$  is 1, X is a heteroatom such as N, O or S. When the linking atom is N, there may be further substitution on the N such as described above for  $R^{10}$ . Specific examples of 1,2,3,4-thiatriazoles are shown below.





The aryldialkylamino disulfides are represented by Formula (D) below.



(D)

In Formula (D), one sulfur atom is bonded directly to a nitrogen atom and the other sulfur atom is bonded to a carbon atom which is part of an aromatic or heteroaromatic ring, Ar. When Ar is an aromatic group, it may be either a single ring or a condensed ring, preferably having 6 to 10 carbon atoms, and more preferably, having 6 carbon atoms. Examples of suitable aromatic groups include phenyl, tolyl, naphthyl, and cycloheptatrienyl. When Ar is a heteroaromatic ring, it may include, for example, pyrrole, pyridine, thiophene, quinoline, benzofuran, pyrazole, oxadiazole, thiadiazole, triazole, tetrazole, benzoxazole, benzothiazole, benzimidazole, or benzotriazole ring systems.

Ar may be further substituted or may be unsubstituted. Examples of suitable substituents include alkyl groups (for example, methyl, ethyl, hexyl), fluoroalkyl groups (for example, trifluoromethyl), alkoxy groups (for example, methoxy, ethoxy, octyloxy), aryl groups (for example, phenyl, naphthyl, tolyl), hydroxy groups, halogen atoms, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl groups (for example, methylsulfonyl, phenylsulfonyl), acylamino groups, sulfonylamino groups, acyloxy groups (for example, acetoxy, benzoxy), carboxy groups, cyano groups, sulfo groups, and amino groups. Preferred are alkyl groups.

R<sup>11</sup> and R<sup>12</sup> are alkyl groups, or together they may form a ring. Examples of such rings include morpholine, piperidine, pyrazolidine, pyrrolidine, and imidazolidine rings. Preferably, the alkyl groups contain 1 to 20 carbon atoms, with 1 to 10 carbon atoms being most preferred. R<sup>11</sup> and R<sup>12</sup> may be substituted as described for Ar.

Specific examples of aryldialkylamino disulfides are shown below.



The sulfur donors of this invention do not include thiosulfonate compounds, particularly those represented by the formula R<sup>13</sup>—SO<sub>2</sub>SM wherein R<sup>13</sup> is an unsubstituted or substituted aliphatic, aromatic or heterocyclic group. Such compounds are further described in Japanese Kokai No. 3-208041, (Waki), filed Jan. 11, 1990, and WO 92/12462, (Lok), filed Dec. 18, 1991. The sulfur donating compounds of this invention also do not include diamino disulfides, particularly those represented by the formula



wherein R<sup>14</sup>, R<sup>15</sup>, R<sup>16</sup> and R<sup>17</sup> are independently hydrogen, or substituted or unsubstituted alkyl, aryl or heterocyclic groups. Such compounds are further described in U.S. application Serial No. 07/890,884, (Lok et al.), filed May 29, 1992.

The preparation of these sulfur donors are known to those skilled in the art and many of them are commercially available.

The sulfonates of this invention are represented by Formula (I),



M (I)

35 Z is a substituted or unsubstituted alkyl, aryl, or heterocyclic group. Preferably, the alkyl groups contain 1 to 20 carbon atoms, with 1 to 10 carbon atoms being most preferred, and the aryl groups contain 6 to 20 carbons atoms and more preferably, 6 to 10 carbon atoms, with 6 carbon atoms being most preferred. The heterocyclic group may be a 5 to 15-membered ring containing one or two heteroatoms. More preferably, the heterocyclic group is a 5 or 6-membered ring. Preferred heteroatoms are nitrogen, oxygen, sulfur, selenium and tellurium, with nitrogen, oxygen, and sulfur being most preferred.

40 Examples of suitable aryl groups include phenyl, tolyl, naphthyl, and cycloheptatrienyl. Examples of suitable heterocyclic groups are pyrrole, furan, tetrahydrofuran, thifuran, pyridine, picoline, piperidine, morpholine, pyrrolidine, thiophene, oxazole, thiazole, imidazole, selenazole, tellurazole, triazole, tetrazole and oxadiazole.

45 Substituents of Z may include, for example, alkyl groups (for example, methyl, ethyl, hexyl), fluoroalkyl groups (for example, trifluoromethyl), alkoxy groups (for example, methoxy, ethoxy, octyloxy), aryl groups (for example, phenyl, naphthyl, tolyl), hydroxy groups, halogen atoms, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl groups (for example, methylsulfonyl, phenylsulfonyl), acylamino groups, sulfonylamino groups, acyloxy groups (for example, acetoxy, benzoxy), carboxy groups, cyano groups, sulfo groups, and amino groups.

50 55 60 65 65 In the most preferred embodiment, Z is an aryl group, and more particularly an unsubstituted phenyl group or a phenyl group substituted in one or two positions.

M is a cationic counter ion. More preferably, M is an alkali metal or ammonium ion, with sodium and potassium ions being most preferred. Examples of suitable sulfonates are shown below.



Many of the sulfonates are commercially available or they may be obtained by reduction of sulfonyl chlorides by methods known to those skilled in the art.

The concentration of sulfur donors and sulfonate compounds which may be utilized covers a wide range. Because of the variety of structures of the sulfur donors and the sulfonate compounds, the levels used will be dependent on the timing of the addition, the layer to which the compounds are added, the type of emulsion and other variables. Those skilled in the art will realize that the balance of the sulfur donor and the sulfonate compound needed to achieve optimal heat stability will vary depending on the desired final product. Generally, the useful concentrations of the sulfur donor are from  $10^{-5}$  to 10 g/mol silver, more preferably, from  $10^{-4}$  to 5 g/mol silver, and most preferably, from  $10^{-3}$  to 1 g/mol silver. Useful concentrations of the sulfonate compound are from  $10^{-4}$  to 100 g/mol silver, more preferably, from  $10^{-3}$  to 50 g/mol silver, and most preferably, from  $10^{-2}$  to 10 g/mol silver. The ratio of sulfur donor to sulfonate compound may vary from 1:0.1 to 1:10.

The sulfur donors and sulfonate compounds may be added to the photographic emulsion using any technique suitable for this purpose. If the sulfur donors or sulfonate compounds are hydrophobic, they may be dissolved in any common organic solvent such as methanol or a mixed aqueous methanolic solution. Examples of other suitable solvents or diluents include ethanol, or acetone. If the sulfur donors or sulfonate compounds are water soluble they can be premixed or they can be added separately in aqueous solutions to the emulsion. The sulfur donors or sulfonate compounds can be added to the emulsion in the form of a liquid/liquid dispersion similar to the technique used with certain couplers. They can also be added as a solid particle dispersion.

The sulfur donor and sulfonate compound may be added to any layer where they are in reactive association with the silver chloride. By "in reactive association with" it is meant that the sulfur donor and the sulfonate compound must be contained in the silver chloride emulsion layer or in a layer whereby they can react or interreact with the silver chloride emulsion. For example, they can also be added to gelatin-only overcoats or interlayers, or to water-only overcoats.

The combination of sulfonates and sulfur donor may be used in addition to any conventional emulsion stabilizer or antifogulant as commonly practiced in the art. Combinations of more than one sulfur donor or sulfonate compound may be utilized.

The photographic emulsions of this invention are generally prepared by precipitating silver halide crystals in a

colloidal matrix by methods conventional in the art. The colloid is typically a hydrophilic film forming agent such as gelatin, alginic acid, or derivatives thereof.

The crystals formed in the precipitation step are chemically and spectrally sensitized, as known in the art. Chemical sensitization of the emulsion employs sensitizers such as sulfur-containing compounds, e.g., allyl isothiocyanate, sodium thiosulfate and allyl thiourea; reducing agents, e.g., polyamines and stannous salts; noble metal compounds, e.g., gold, platinum; and polymeric agents, e.g., polyalkylene oxides. A temperature rise is employed to complete chemical sensitization (heat treatment). Spectral sensitization is effected with agents such as sensitizing dyes. For color emulsions, dyes are added in the spectral sensitization step using any of a multitude of agents described in the art. It is known to add such dyes both before and after heat treatment.

After spectral sensitization, the emulsion is coated on a support. Various coating techniques include dip coating, air knife coating, curtain coating and extrusion coating.

The sulfur donors and sulfonate compounds of this invention may be added to the silver halide emulsion at any time during the preparation of the emulsion, i.e., during precipitation, during or before chemical sensitization or during final melting and co-mixing of the emulsion and additives for coating. Most preferably, these compounds are added after chemical sensitization. The sulfur donor and the sulfonate compound do not have to be added simultaneously, and they may be added at different points in the preparation of the emulsion. Preferably, the sulfonate compound is added first followed by the sulfur donor.

The photographic elements of this invention can be any photographic recording material comprising, at least one high chloride silver emulsion. The other emulsions of the photographic element may have any halide content. For example, the photographic element may also contain silver bromide or silver iodobromide emulsions. The silver chloride emulsion must be comprised of greater than 50 mole percent, and more preferably, greater than 90 mole percent silver chloride.

The photographic elements of this invention can be non-chromogenic silver image forming elements. They can be single color elements or multicolor elements. Multicolor elements typically contain dye image-forming units sensitive to each of the three primary regions of the visible spectrum. Each unit can be comprised of a single emulsion layer or of multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer, e.g., as by the use of microvessels as described in Whitmore U.S. Pat. No. 4,362,806 issued Dec. 7, 1982. The element can contain additional layers such as filter layers, interlayers, overcoat layers, subbing layers and the like. This invention may be particularly useful with those photographic elements containing a magnetic backing such as described in No. 34390, *Research Disclosure*, Nov. 1992.

In the following discussion of suitable materials for use in the emulsions and elements of this invention, reference will be made to *Research Disclosure*, Dec. 1989, Item 308119, published by Kenneth Mason Publications, Ltd., Dudley Annex, 12a North Street, Emsworth, Hampshire PO10 7DQ, ENGLAND, the disclosures of which are incorporated herein by reference. This publication will be identified hereafter by the term "Research Disclosure".

## 11

The silver halide emulsions employed in the elements of this invention can be either negative-working or positive-working. Examples of suitable emulsions and their preparation are described in Research Disclosure Sections I and II and the publications cited therein. Other suitable emulsions are (111) tabular silver chloride emulsions such as described in U.S. Pat. Nos. 5,176,991 (Jones et al); 5,176,992 (Maskasky et al); 5,178,997 (Maskasky); 5,178,998 (Maskasky et al); 5,183,732 (Maskasky); and 5,185,239 (Maskasky) and (100) tabular silver chloride emulsions such as described in EP 0 534,395, published Mar. 31, 1993 (Brust et al). Some of the suitable vehicles for the emulsion layers and other layers of elements of this invention are described in Research Disclosure Section IX and the publications cited therein.

The silver halide emulsions can be chemically and spectrally sensitized in a variety of ways, examples of which are described in Sections III and IV of the Research Disclosure. The elements of this invention can include various dye-forming couplers including but not limited to those described in Research Disclosure Section VII, paragraphs D, E, F and G and the publications cited therein. These couplers can be incorporated in the elements and emulsions as described in Research Disclosure Section VII, paragraph C and the publications cited therein.

The photographic elements of this invention or individual layers thereof can contain, among other things, brighteners (Examples in Research Disclosure Section V), antifoggants and stabilizers (Examples in Research Disclosure Section VI), antistain agents and image dye stabilizers (Examples in Research Disclosure Section VII, paragraphs I and J), light absorbing and scattering materials (Examples in Research Disclosure Section VIII), hardeners (Examples in Research Disclosure Section X), plasticizers and lubricants (Examples in Research Disclosure Section XII), antistatic agents (Examples in Research Disclosure Section XIII), matting agents (Examples in Research Disclosure Section XVI) and development modifiers (Examples in Research Disclosure Section XXI).

The photographic elements can be coated on a variety of supports including but not limited to those described in Research Disclosure Section XVII and the references described therein.

Photographic elements can be exposed to actinic radiation, typically in the visible region of the spectrum, to form a latent image as described in Research Disclosure Section XVIII and then processed to form a visible dye image examples of which are described in Research Disclosure Section XIX. Processing to form a visible dye image includes the step of contacting the element with a color developing agent to reduce developable silver halide and oxidize the color developing agent. Oxidized color developing agent in turn reacts with the coupler to yield a dye.

With negative working silver halide, the processing step described above gives a negative image. To obtain a positive (or reversal) image, this step can be preceded by development with a non-chromogenic developing agent to develop exposed silver halide, but not form dye, and then uniformly fogging the element to render unexposed silver halide developable, and then developed with a color developer. Additionally, the preceding process can be employed but before uniformly fogging the emulsion the remaining silver halide is dissolved and the developed silver is converted back to silver halide; the conventional E-6 process is then continued and results in a negative color image. Alternatively, a direct positive emulsion can be employed to obtain a positive image.

## 12

Development is followed by the conventional steps of bleaching, fixing, or bleach-fixing, to remove silver and silver halide, washing and drying.

The following examples are intended to illustrate, without limiting, this invention.

## EXAMPLES

## Example 1

A chemically and blue spectrally sensitized monodisperse silver chloride negative emulsion having yellow dye-forming coupler  $\alpha$ -(4-(4-benzyloxy-phenyl-sulfonyl)phenoxy)- $\alpha$ (pivalyl)-2-chloro-5-( $\gamma$ -(2,4-di-5-amylphenoxy)butyramido)acetanilide (1.08 g/m<sup>2</sup>) in di-n-butylphthalate coupler solvent (0.27 g/m<sup>2</sup>) and gelatin (1.51 g/m<sup>2</sup>) was prepared. In addition, 0.104 g of 1(3-acetamidophenyl)-5-mercaptopotetrazole and 1.033 g of potassium bromide per silver mole were added. The emulsion was divided and various concentrations of a methanolic solution of either the compounds C1, C3 or C5 and/or a methanolic solution of S3, were added to the different portions. The emulsions (0.34 g Ag/m<sup>2</sup>) were coated on resin coated paper supports and 1.076 g/m<sup>2</sup> gel overcoat was applied as a protective layer along with the hardener bis (vinylsulfonyl) methyl ether in an amount of 1.8% of the total gelatin weight. The coatings were stored at 0° F. and 120° F. and 50% relative humidity for two weeks.

The coatings were given a 0.1 second exposure, using a 0-3 step tablet (0.15 increments) with a tungsten lamp designed to simulate a color negative print exposure source. This lamp had a color temperature of 3000 K, log lux 2.95, and the coatings were exposed through a combination of magenta and cyan filters, a 0.3 ND (Neutral Density), and a UV filter. The processing consisted of color development (45 sec, 35° C.), bleach-fix (45 sec, 35° C.) and stabilization or water wash (90 sec, 35° C.) followed by drying (60 sec, 60° C.). The chemistry used in the Colenta processor consisted of the following solutions:

| Developer:                                                                                                          |         |
|---------------------------------------------------------------------------------------------------------------------|---------|
| Lithium salt of sulfonated polystyrene                                                                              | 0.25 mL |
| Triethanolamine                                                                                                     | 11.0 mL |
| N,N-diethylhydroxylamine (85% by wt.)                                                                               | 6.0 mL  |
| Potassium sulfite (45% by wt.)                                                                                      | 0.5 mL  |
| Color developing agent (4-(N-ethyl-N-2-methanesulfonyl aminoethyl)-2-methyl-phenylenediaminesquisulfate monohydrate | 5.0 g   |
| Stilbene compound stain reducing agent                                                                              | 2.3 g   |
| Lithium sulfate                                                                                                     | 2.7 g   |
| Acetic acid                                                                                                         | 9.0 mL  |
| Water to total 1 liter, pH adjusted to                                                                              | 6.2     |
| Potassium chloride                                                                                                  | 2.3 g   |
| Potassium bromide                                                                                                   | 0.025 g |
| Sequestering agent                                                                                                  | 0.8 g   |
| Potassium carbonate                                                                                                 | 25.0 g  |
| Water to total of 1 liter, pH adjusted to                                                                           | 10.12   |
| Bleach-fix                                                                                                          |         |
| Ammonium sulfite                                                                                                    | 58 g    |
| Sodium thiosulfate                                                                                                  | 8.7 g   |
| Ethylenediaminetetraacetic acid ferric ammonium salt                                                                | 40 g    |
| Stabilizer                                                                                                          |         |
| Sodium citrate                                                                                                      | 1 g     |
| Water to total 1 liter, pH adjusted to                                                                              | 7.2     |

The speed at 1.0 density unit was taken as a measure of the sensitivity of the emulsion. Heat sensitivity data was obtained on a sensitometer which was modified with a water

jacket so that the temperature of the step tablet could be maintained at 22° C. or increased to 40° C. A 0.1 second exposure was made with a 3000 K light source and the coatings were processed with RA-4 chemistry. The change in speed due to the temperature variation ( $\Delta$ speed) was calculated at the 1.0 density point of the D log E curve and is shown in Table I.

Table I also illustrates the changes in fog ( $\Delta$ fog) due to storage for 2 weeks at 120° F. and 50% relative humidity.

TABLE I

| Compound | mg Ag mole | S3 | Sample #       | 2 week                           |                                    | Heat Sensitivity<br>40° C. vs 22° C.<br>$\Delta$ Speed |
|----------|------------|----|----------------|----------------------------------|------------------------------------|--------------------------------------------------------|
|          |            |    |                | 120° F. vs 0° F.<br>$\Delta$ Fog | 40° C. vs 22° C.<br>$\Delta$ Speed |                                                        |
| 0        | 0          | —  | 1 (comparison) | 0.83                             | 4                                  |                                                        |
| 0        | 0          | +  | 2 (comparison) | 0.80                             | 3                                  |                                                        |
| C1       | 70         | —  | 3 (comparison) | 0.53                             | -4                                 |                                                        |
| C1       | 70         | +  | 4 (invention)  | 0.55                             | 1                                  |                                                        |
| C3       | 91         | —  | 5 (comparison) | 0.13                             | -13                                |                                                        |
| C3       | 91         | +  | 6 (invention)  | 0.18                             | -8                                 |                                                        |
| C5       | 78         | —  | 7 (comparison) | 0.32                             | -7                                 |                                                        |
| C5       | 78         | +  | 8 (invention)  | 0.45                             | -3                                 |                                                        |

S3 is coated at 10x weight of Compounds C.

mole, respectively. The data in Table II shows the changes in fog ( $\Delta$ fog) and heat sensitivity.

It can be seen that the thiatriazoles reduce fog growth due to storage relative to the control (samples 3, 4, 5, 6, 7, and 8 relative to sample 1). Coatings containing only thiatriaz-

TABLE II

| Compound | mg Ag mole | S3 | Sample #        | 2 week                           |                                    | Heat Sensitivity<br>40° C. vs 22° C.<br>$\Delta$ Speed |
|----------|------------|----|-----------------|----------------------------------|------------------------------------|--------------------------------------------------------|
|          |            |    |                 | 120° F. vs 0° F.<br>$\Delta$ Fog | 40° C. vs 22° C.<br>$\Delta$ Speed |                                                        |
| 0        | 0          | —  | 9 (comparison)  | 0.31                             | 8                                  |                                                        |
| C1       | 109        | —  | 10 (comparison) | 0.20                             | 3                                  |                                                        |
| C1       | 109        | +  | 11 (invention)  | 0.21                             | 7                                  |                                                        |
| C1       | 273        | —  | 12 (comparison) | 0.13                             | -4                                 |                                                        |
| C1       | 273        | +  | 13 (invention)  | 0.14                             | 4                                  |                                                        |
| C2       | 100        | —  | 14 (comparison) | 0.27                             | 4                                  |                                                        |
| C2       | 100        | +  | 15 (invention)  | 0.29                             | 7                                  |                                                        |
| C2       | 250        | —  | 16 (comparison) | 0.26                             | 1                                  |                                                        |
| C2       | 250        | +  | 17 (invention)  | 0.25                             | 7                                  |                                                        |
| C6       | 134        | —  | 18 (comparison) | 0.22                             | 3                                  |                                                        |
| C6       | 134        | +  | 19 (invention)  | 0.19                             | 5                                  |                                                        |
| C6       | 335        | —  | 20 (comparison) | 0.18                             | -1                                 |                                                        |
| C6       | 335        | +  | 21 (invention)  | 0.12                             | 1                                  |                                                        |

S3 is coated at 10x weight of the thiatriazoles

oles (samples 3, 5, and 7) cause the heat sensitivity change to go negative, an equally undesirable position. However, coatings with the combination (samples 4, 6, and 8) have smaller changes in heat sensitivity but still reduce fog growth. It can also be seen that S3 alone in the coating (sample 2) has little effect on either the keeping or the heat sensitivity properties of the emulsion.

#### Example 2

This example demonstrates the beneficial effect of the combination of thiatriazoles and S3 in a red sensitized emulsion prepared as in Example 1 except the emulsion was coated at 0.18 g Ag/m<sup>2</sup>, and the cyan dye-forming coupler 2-( $\alpha$ -(2,4-di-tert-ethyl-phenoxy)butyramido)-4,6-dichloro-5-ethyl phenol (0.42 g/m<sup>2</sup>) in di-n-butyl phthalate coupler solvent (0.429 g/m<sup>2</sup>) and gelatin (1.08g/m<sup>2</sup>) were used. The amounts of 1-(3-acetamidophenyl)-5-mercaptotetrazole and potassium bromide were changed to 0.38 and 1.1 g per silver

It can be seen in Table II that all coatings with thiatriazoles (samples 10-21) reduce fog growth and heat sensitivity of the emulsion relative to the control (sample 9). Depending on the thiatriazoles and the levels used, the combination with sulfinate, S3 (e.g. sample 21) demonstrates that the sulfinate moves the heat sensitivity in a positive direction and still effectively reduces fog growth.

#### Example 3

This experiment shows the effect of the combination of the thiepin, B1, and S3 in an emulsion prepared as in Example 2. The emulsions were stored at 0° F. and at 120° F. for one week and two weeks and then exposed and processed as described above. The data in Table III shows the changes and heat sensitivity.

TABLE III

| B1<br>mg<br>Ag mole | S3<br>mg<br>Ag mole | 1 week<br>120° F. vs 0° F.<br>ΔFog | 2 week<br>120° F. vs 0° F.<br>ΔFog | Heat Sensitivity<br>40° C. vs 22° C.<br>ΔSpeed |
|---------------------|---------------------|------------------------------------|------------------------------------|------------------------------------------------|
| control             | 0 22 (comparison)   | 0.06                               | 0.12                               | 7                                              |
| 0                   | 400 23 (comparison) | 0.05                               | 0.11                               | 7                                              |
| 20                  | 0 24 (comparison)   | 0.01                               | 0.04                               | -8                                             |
| 20                  | 200 25 (invention)  | 0.03                               | 0.06                               | 4                                              |
| 40                  | 0 26 (comparison)   | 0.01                               | 0.03                               | -9                                             |
| 40                  | 400 27 (invention)  | 0.02                               | 0.04                               | 3                                              |

Table III shows that B1 significantly reduces fog growth during incubation (samples 24 and 26), but that the heat sensitivity has moved in the negative direction. The combination of B1 and S3 (e.g. sample 27) reduces the speed change from heat sensitivity but still maintains the antifogging property of B1 alone.

#### Example 4

This example demonstrates the beneficial effect of the combination of S3 and A1 in a red sensitized 5 emulsion prepared as in example 2. The emulsions were stored at 0° F. and at 140° F. for one week and at 0° F. and at 120° F. for two weeks and then exposed and processed as described above. The data in Table IV shows the change in fog (Δfog) and heat sensitivity.

TABLE IV

| A1<br>mg<br>Ag mole | S3<br>mg<br>Ag mole | 1 week<br>140° F. vs 0° F.<br>ΔFog | 2 week<br>120° F. vs 0° F.<br>ΔFog | Heat Sensitivity<br>40° C. vs 22° C.<br>ΔSpeed |
|---------------------|---------------------|------------------------------------|------------------------------------|------------------------------------------------|
| 0                   | 0 28 (comparison)   | 0.15                               | 0.65                               | 6                                              |
| 0                   | 150 29 (comparison) | 0.14                               | 0.71                               | 6                                              |
| 5                   | 0 30 (comparison)   | 0.12                               | 0.05                               | 2                                              |
| 5                   | 50 31 (invention)   | 0.10                               | 0.05                               | 4                                              |
| 15                  | 0 32 (comparison)   | 0.07                               | 0.03                               | -5                                             |
| 15                  | 150 33 (invention)  | 0.06                               | 0.03                               | 0                                              |

It can be seen in Table IV that a coating containing the combination of sulfinate, S3 and a sulfur releasing agent, A1, (sample 33) has smaller fog increase and smaller change in speed when exposed at high temperature than either one of the additives by themselves (samples 29, 30, and 32) or the control (sample 28).

#### Example 5

This experiment shows the beneficial effects of the combination of sulfinate, S3 and a vulcanizing agent, D1 in an emulsion prepared and processed as in Example 1. The data in Table V shows the changes in fog and heat sensitivity.

TABLE V

| B1<br>mg<br>Ag mole | S3<br>mg<br>Ag mole  | 1 week<br>120° F. vs 0° F.<br>ΔFog | Heat Sensitivity<br>40° C. vs 22° C.<br>ΔSpeed(2) |
|---------------------|----------------------|------------------------------------|---------------------------------------------------|
| 0                   | 0 34 (comparison)    | 0.18                               | 7                                                 |
| 0                   | 9000 35 (comparison) | 0.18                               | 6                                                 |
| 125                 | 0 36 (comparison)    | 0.07                               | -4                                                |
| 125                 | 9000 37 (invention)  | 0.08                               | 3                                                 |
| 188                 | 0 38 (comparison)    | 0.07                               | -7                                                |
| 188                 | 9000 39 (invention)  | 0.07                               | -1                                                |
| 250                 | 0 40 (comparison)    | 0.08                               | -8                                                |
| 250                 | 9000 41 (invention)  | 0.05                               | -1                                                |

All of the coatings containing D1 show significantly lower fog growth than the coatings without. Upon exposure at high temperature, the control (sample 34) has increased speed, but the coatings containing D1 alone actually show decreased speed (samples 36, 35 and 40). However, the coatings with S3 and D1 (samples 37, 39, and 41) show much less change in heat sensitivity and lower fog growth.

#### Example 6

In this example the beneficial effect of the combination of D1 and S3 is seen in a red sensitized emulsion prepared and processed as in Example 2. The data in Table VI shows the changes in fog and heat sensitivity.

TABLE VI

| B1<br>mg<br>Ag mole | S3<br>mg<br>Ag mole  | 1 week<br>120° F. vs 0° F.<br>ΔFog | Heat Sensitivity<br>40° C. vs 22° C.<br>ΔSpeed |
|---------------------|----------------------|------------------------------------|------------------------------------------------|
| 0                   | 0 42 (comparison)    | 0.12                               | 7                                              |
| 0                   | 4800 43 (comparison) | 0.12                               | 6                                              |
| 25                  | 0 44 (comparison)    | 0.09                               | -1                                             |
| 25                  | 500 45 (invention)   | 0.08                               | 2                                              |
| 50                  | 0 46 (comparison)    | 0.07                               | -6                                             |
| 50                  | 1000 47 (invention)  | 0.06                               | 2                                              |
| 75                  | 0 48 (comparison)    | 0.07                               | -7                                             |
| 75                  | 1500 49 (invention)  | 0.05                               | 1                                              |
| 100                 | 0 50 (comparison)    | 0.06                               | -9                                             |
| 100                 | 2000 51 (invention)  | 0.04                               | -1                                             |
| 125                 | 0 52 (comparison)    | 0.08                               | -11                                            |
| 125                 | 2500 53 (invention)  | 0.03                               | -2                                             |

Table VI shows the reduction in fog after incubation for 60 coatings that contain D1 (samples 44-53) relative to the two coatings without (samples 42,43). However, the coatings with only D1 (samples 44, 46, 48, 50, and 52) show a negative change in speed on exposure at high temperature. The coatings with both D1 and S3 (samples 45, 47, 49, 51, and 53) show the least change in speed upon exposure at elevated temperature relative to the control.

## Example 7

This experiment shows the effect of the combination of elemental sulfur, ES, and S3 on fog and heat sensitivity in a blue sensitized emulsion prepared as in Example 1. The emulsions were stored at 0 °F. and at 140° F. for three days and at 0° F. and at 120° F. for two weeks and then exposed and processed as described above. The data in Table VII shows the changes in fog and heat sensitivity.

TABLE VII

| ES<br>mg<br>Ag mole | S3<br>mg<br>Sample # | 3 day<br>140° F. vs 0° F.<br>ΔFog | 2 week<br>120° F. vs 0° F.<br>ΔFog | Heat Sensitivity<br>40° C. vs 22° C.<br>ΔSpeed |
|---------------------|----------------------|-----------------------------------|------------------------------------|------------------------------------------------|
| 0                   | 0 54 (comparison)    | 0.32                              | 0.83                               | 3                                              |
| 0                   | 2400 55 (comparison) | 0.33                              | 0.80                               | 3                                              |
| 0.5                 | 0 56 (comparison)    | 0.22                              | 0.65                               | -4                                             |
| 0.5                 | 500 57 (invention)   | 0.30                              | 0.71                               | 2                                              |
| 1.0                 | 0 58 (comparison)    | 0.17                              | 0.44                               | -10                                            |
| 1.0                 | 500 59 (invention)   | 0.23                              | 0.52                               | 0                                              |
| 1.5                 | 0 60 (comparison)    | 0.14                              | 0.34                               | -12                                            |
| 1.5                 | 500 61 (invention)   | 0.21                              | 0.56                               | -1                                             |

Samples 56–61 containing ES have reduced fog compared to the samples without (54 and 55). While the control (sample 54) shows an increase in speed upon exposure to high temperature, the coatings containing only ES show a decrease in heat sensitivity. The coatings containing the combinations (samples 57, 59, and 61) show the least change in speed on exposure to 40° C., while the fog increase after storage is still less than that of the control. Again, the coating containing S3 alone (sample 55) has no effect on either heat sensitivity or fog.

## Example 8

In this experiment the beneficial effect of the combination of ES and S3 is seen in a red sensitized emulsion prepared and processed as in Example 2. The data in Table VIII shows the changes in fog and heat sensitivity.

TABLE VIII

| ES<br>mg<br>Ag mole | S3<br>mg<br>Sample # | 1 week<br>120° F. vs 0° F.<br>ΔFog | Heat Sensitivity<br>40° C. vs 22° C.<br>ΔSpeed(2) |
|---------------------|----------------------|------------------------------------|---------------------------------------------------|
| 0                   | 0 62 (comparison)    | 0.22                               | 7                                                 |
| 0                   | 100 63 (comparison)  | 0.22                               | 7                                                 |
| 0.1                 | 0 64 (comparison)    | 0.19                               | 3                                                 |
| 0.1                 | 100 65 (invention)   | 0.20                               | 5                                                 |
| 0.3                 | 0 66 (comparison)    | 0.17                               | -3                                                |
| 0.3                 | 100 67 (invention)   | 0.18                               | 2                                                 |
| 0.5                 | 0 68 (comparison)    | 0.17                               | -4                                                |
| 0.5                 | 100 69 (invention)   | 0.16                               | 1                                                 |

It can be seen that the coatings containing ES (samples 64–67) have reduced fog growth compared to the coatings without ES (samples 62 and 63). While the control (sample 62) shows an increase in speed upon exposure to high temperature, the coatings containing ES show a decrease in heat sensitivity. The coatings containing the preferred ES and S3 combination (samples 67 and 69) show the least change in speed, but with fog growth still less than the

control (sample 62). Sample 63 which contains only S3 shows no effect on either heat sensitivity or fog.

## Example 9

This example shows that certain sulfur extruding compounds are much less effective in reducing fog growth and heat sensitivity. 1,4-dithiins are known to extrude sulfur on heating, and depending on the substituents on the dithiin ring, may require a temperature of around 200° C. for ring contraction. Table IX shows the data for two dithiins, M1 and M2 in an emulsion prepared as in example 2.

TABLE IX

| Compound | mg Ag mole | Sample #        | 3 day                    | 2 week                   | Heat Sensitivity           |
|----------|------------|-----------------|--------------------------|--------------------------|----------------------------|
|          |            |                 | 140° F. vs 0° F.<br>ΔFog | 120° F. vs 0° F.<br>ΔFog | 40° C. vs 22° C.<br>ΔSpeed |
| 0        | 0          | 70 (comparison) | 0.07                     | 0.08                     | 7                          |
| M1       | 1.6        | 71 (invention)  | 0.07                     | 0.08                     | 6                          |
| M1       | 32         | 72 (invention)  | 0.05                     | 0.07                     | 5                          |
| M2       | 1.8        | 73 (invention)  | 0.06                     | 0.04                     | 5                          |
| M2       | 35         | 74 (invention)  | 0.04                     | 0.03                     | 6                          |

It can be seen that the dithiins are somewhat effective in reducing fog growth, but are only slightly active in depressing heat sensitivity.

#### Example 10

In this example an emulsion was prepared as described in Example 6, except the disulfides were replaced with two other disulfides, M3 and M4, that are not sulfur donors and are outside of the scope of this invention. The data in Table X shows the change in fog and heat sensitivity.

20 mole % silver chloride, said emulsion being in reactive association with a sulfur donating compound, and a sulfinate compound represented by Formula (I)



wherein Z is a non-metallic aryl, alkyl or heterocyclic group, and M is a cationic counter ion; and wherein the sulfur donating compound is selected from the group consisting of a disulfide, polysulfide,

TABLE X

| Compound | mg Ag mole | Sample #        | 1 week                   | Heat Sensitivity        |
|----------|------------|-----------------|--------------------------|-------------------------|
|          |            |                 | 120° F. vs 0° F.<br>ΔFog | 40° vs 22° C.<br>ΔSpeed |
| none     | 0          | 75 (comparison) | 0.16                     | 9                       |
| none     | 0          | 76 (comparison) | 0.14                     | 10                      |
| M3       | 448        | 0               | 0.14                     | 11                      |
| M3       | 448        | 78 (comparison) | 0.16                     | 10                      |
| M4       | 180        | 0               | 0.18                     | 8                       |
| M4       | 180        | 2,400           | 0.15                     | 9                       |

It can be seen from Table X that the two disulfides, M3 and M4, offer little protection against the effects of storage 50 and heat sensitivity reduction with or without a sulfinate.

In summary, the keeping and the heat sensitivity properties of silver chloride emulsions can clearly be modified by elemental sulfur, sulfur donating compounds and sulfinites. Depending on the levels of these materials used, the ratio of sulfur donors to sulfinites and the nature of the sulfur precursors, those skilled in the art can optimize each of these parameters to best suit the needs of the photographic emulsions and applications.

While the invention has been described in detail and with reference to specific embodiments thereof, it will be apparent to one skilled in the art that various changes and modifications can be made therein without departing from the spirit and scope thereof.

What is claimed is:

1. A negative silver halide photographic element comprising a silver halide emulsion which is greater than 90

sulfenic sulfonic thioanhydride, acylmethylmercapto azole, acylmethylmercapto azolium salt, thiazepine, thiepin, 1,4dithiin, 1,2-thiazine, 1,3-thiazine, 1,4-thiazine, 1,4,2-dithiazine, 1,3,4-thiadiazine, 1,2,6-thiadiazine, 1,3,5-thiadiazine, benzothiazolyl-2-N-dithiomorpholide, and elemental sulfur dissolved in an alcoholic solvent; and

wherein the sulfur donating compound is not a diamino disulfide.

2. The photographic element of claim 1 wherein Z is an alkyl group of 1 to 20 carbon atoms, an aryl group of 6 to 20 carbon atoms or a heterocyclic group of 5 to 15 members with at least one atom selected from nitrogen, oxygen, sulfur, selenium and tellurium, and M is an alkali metal or ammonium ion.

3. The photographic element of claim 2 wherein Z is an alkyl group of 1 to 10 carbon atoms, an aryl group of 6 to 10 carbon atoms or a heterocyclic group of 5 to 6 members

## 21

with at least one atom selected from nitrogen, oxygen, and sulfur, and M is an alkali metal ion.

4. The photographic element of claim 3 wherein Z is an aryl group, and M is sodium or potassium.

5. The photographic element of claim 1 wherein the sulfur donating compound is an aryldialkylamino disulfide, an acylmethylmercapto azonium salt, elemental sulfur dissolved in an alcoholic solvent or a thiepin.

6. The photographic element of claim 1 wherein the concentration of the sulfur donating compound is from  $10^{-3}$  to 1 g/mol Ag and the concentration of the sulfinate compound is from  $10^{-2}$  to 10 g/mol Ag.

7. The photographic element of claim 1 wherein the sulfur donating compound is an aryldialkylamino disulfide, an acylmethylmercapto azonium salt, or a thiepin;

Z is an alkyl group of 1 to 20 carbon atoms, an aryl group of 6 to 20 carbon atoms or a heterocyclic group of 5 to 15 members with at least one atom selected from nitrogen, oxygen, sulfur, selenium and tellurium, and M is an alkali metal or ammonium ion; and

the concentration of sulfur donating compound is from  $10^{-3}$  to 1 g/mol Ag; and the concentration of sulfinate compound is from  $10^{-2}$  to 10 g/mol Ag.

8. The photographic element of claim 7 wherein Z is an alkyl group of 1 to 10 carbon atoms, an aryl group of 6 to 10 carbon atoms or a heterocyclic group of 5 to 6 members with at least one atom selected from nitrogen, oxygen, and sulfur, and M is an alkali metal ion.

9. A method of making a negative silver halide emulsion which is greater than 90 mole % silver chloride, comprising precipitating and chemically sensitizing the emulsion and further comprising adding to the emulsion a sulfur donating compound and a sulfinate compound represented by Formula II



wherein Z is a non-metallic aryl, alkyl or heterocyclic group, and M is a cationic counter ion;

wherein the sulfur donating compound is selected from the group consisting of a disulfide, polysulfide, sulfenic sulfonic thioanhydride, acylmethylmercapto azole, acylmethylmercapto azonium salt, thiazepine, thiepin,

## 22

1,4-dithiin, 1,2-thiazine, 1,3-thiazine, 1,4-thiazine, 1,4,2-dithiazine, 1,3,4-thiadiazine, 1,2,6-thiadiazine, 1,3,5-thiadiazine, benzothiazolyl-2-N-dithiomorpholide, and elemental sulfur dissolved in alcoholic solvent; and wherein the sulfur donating compound is not a diamino disulfide.

10. The method of claim 9 wherein Z is an alkyl group of 1 to 20 carbon atoms, an aryl group of 6 to 20 carbon atoms or a heterocyclic group of 5 to 15 members with at least one atom selected from nitrogen, oxygen, sulfur, selenium and tellurium, and M is an alkali metal or ammonium ion.

11. The method of claim 10 wherein Z is an alkyl group of 1 to 10 carbon atoms, an aryl group of 6 to 10 carbon atoms or a heterocyclic group of 5 to 6 members with at least one atom selected from nitrogen, oxygen, and sulfur, and M is an alkali metal ion.

12. The method of claim 11 wherein Z is an aryl group, and M is sodium or potassium.

13. The method of claim 9 wherein the sulfur donating compound is an aryldialkylamino disulfide, an acylmethylmercapto azonium salt or a thiepin.

14. The method of claim 9 wherein the amount of sulfur donating compound added is from  $10^{-3}$  to 1 g/mol Ag and the amount of the sulfinate compound added is from  $10^{-2}$  to 10 g/mol Ag.

15. The method of claim 9 wherein the sulfur donating compound is an aryldialkylamino disulfide, an acylmethylmercapto azonium salt or a thiepin;

Z is an alkyl group of 1 to 20 carbon atoms, an aryl group of 6 to 20 carbon atoms or a heterocyclic group of 5 to 15 members with at least one atom selected from nitrogen, oxygen, sulfur, selenium and tellurium, and M is an alkali metal or ammonium ion;

the amount of sulfur donating compound added is from  $10^{-3}$  to 1 g/mol Ag; and the amount of sulfinate compound added is from  $10^{-2}$  to 10 g/mol Ag.

16. The method of claim 15 wherein Z is an alkyl group of 1 to 10 carbon atoms, an aryl group of 6 to 10 carbon atoms or a heterocyclic group of 5 to 6 members with at least one atom selected from nitrogen, oxygen, and sulfur, and M is an alkali metal ion.

\* \* \* \* \*